

E. R. VIBERG.

**METHOD OF MAKING BRAKE BEAM FULCRUMS,  
APPLICATION FILED MAY 31, 1919.**

1,414,607.

Patented May 2, 1922.



# UNITED STATES PATENT OFFICE.

ERNEST R. VIBERG, OF MONTREAL, QUEBEC, CANADA, ASSIGNOR TO CANADIAN CAR AND FOUNDRY COMPANY LIMITED, OF MONTREAL, QUEBEC, CANADA, A CORPORATION.

## METHOD OF MAKING BRAKE-BEAM FULCRUMS.

1,414,607.

Specification of Letters Patent.

Patented May 2, 1922.

Application filed May 31, 1919. Serial No. 301,073.

To all whom it may concern:

Be it known that I, ERNEST R. VIBERG, a subject of the King of Great Britain, and resident of the city of Montreal, in the Province of Quebec and Dominion of Canada, have invented certain new and useful Improvements in Methods of Making Brake-Beam Fulcrums, of which the following is a full, clear, and exact description.

10 This invention relates to improvements in forged brake beam fulcrums and in the method of making same, and the object of the invention is to provide a forged fulcrum of very light weight which will have the required stiffness and bearing surface for the fulcrum pin and which may be made very easily and cheaply.

At the present time, owing to the increased service required of brake beam fulcrums on account of the increased weight and capacity of cars, it has been found that cast fulcrums are not reliable when made within the permissible limits of weight and size, and there is therefore demand for a 25 forged fulcrum which will combine the necessary strength with a minimum of size and weight and with low cost.

According to the present invention, a fulcrum is produced in which the cross section 30 of material is varied in the different parts of the fulcrum according to requirements, so that the necessary strength may be obtained where required not accompanied by an unnecessary body of material where as great 35 strength is not necessary. In order to produce this result, a bar of metal is elongated by a rough drawing or forging operation, which serves to distribute the metal in varying amounts at different points in the length 40 of the bar. This bar is then forged to the desired shape and finally bent to its finished form. The method of forging differs from that previously employed in that the bending of the bar to its final new form is one of 45 the last operations, whereas according to previous methods the bending has been one of the first operations. The result is that according to this invention, the forgings

are carried out on a flat bar and therefore much more easily than when the bar is bent. 50

In the drawings which illustrate the invention:

Fig. 1 is a plan view of a bar after the first rough drawing or forging operation.

Fig. 2 is a plan view of the bar after the 55 final forging operation.

Fig. 3 is an edge elevation corresponding to Figure 2.

Fig. 4 is a plan view of the fulcrum complete. 60

Figs. 5 and 6 are fragmentary plan views showing alternative foot constructions for the fulcrum.

Referring more particularly to the drawings, 11 designates a bar of metal, rough 65 forged to provide a central enlargement 12 and two other enlargements 13 located one on either side of the central enlargement 12 and equidistant therefrom. Beyond the enlargements 13, the bar is reduced to a point 70 near the ends and the end portions 14 are offset to opposite sides of the bar. In the next forging operation, the central portion 12 is driven out of the plane of the bar, as clearly shown in Figure 3, so as to form the 75 actual U-bend 15 at the end of the fulcrum and also the seat 16 for the tension member of the brake beam. It will be noted that the bend or end of the fulcrum is now out of the plane of the bar, which has become divided into arms 17 connected to the end of the fulcrum at the bends 18 and lying in alignment. Each of the enlargements 13 is increased in size, as shown at 19, and pockets 20 are formed in opposite sides of each 80 arm concentric with the enlargements 19. The metal displaced in the formation of these pockets forms a boss 21 on the same side of the bar on which the U-bend 15 lies. These bosses add to the thickness of the 85 arms 17 sufficiently to give the required bearing surfaces for the fulcrum pin. At the same time that the bosses 21 are formed, ribs 22 are produced on each side of each boss extending in the longitudinal direction 90 of the arms and serve to stiffen the arms

60

75

80

85

95

adjacent the boss and U-bend. At the next operation, each arm 17 is twisted through approximately 45° adjacent its free end, as clearly shown at 23, Figure 4, and is then bent beyond the twist through an angle of 90° to form feet 24, by means of which the fulcrum may be secured to the compression member of a brake beam. The final operation of forming the beam is to straighten out the bends 18, thus bringing the two arms into parallelism, as shown in Figure 4. The fulcrum is now finished by drilling through at the pockets 20 to receive a fulcrum pin and through the feet to receive attaching rivets. From the foregoing description, it will be seen that all the forging operations are carried out on a substantially flat bar, so that the dies may be of the simplest character. The whole process of manufacture is infinitely more simple than the existing processes, in which the bar is first bent to new form and is afterwards forged to form the socket 16 and twisted to bring the arms into proper angular relation with the feet. It is obvious that the operation of forging the socket and twisting to properly dispose the feet is greatly complicated by the U form of the bar and that quite elaborate gripping dies are necessary in addition to the forging dies.

While the arms have been shown separate at their foot ends in Figure 4, it will be understood that the invention is not limited to this feature, as the free extremities of the arms may be drawn together at their twisted points 23 and welded together into a bar 25, as in Figure 5, or when drawn together may be welded or riveted to form a flat bar 26, as in Figure 6. After forming into either of the forms shown in Figures 5 or 6, the feet 24 are turned outwardly for attachment to the compression member of a brake beam. It will be understood that if desired the feet of the fulcrum in the form shown in Figure 4 may be formed after the arms have been bent into parallelism.

It will be noted that in any of the forms, the ends of the bar are oppositely offset. This offsetting facilitates forming the twists 50 23 in the arms and reduces stresses in the metal which would be caused if the arms were straight by the greater stretching of one edge to bring the edges of the bar between the twists and the extremities into 55 alignment.

Between the fulcrum pin and the feet of the fulcrum there is no great load on the fulcrum, so that much less metal is required in this part of the bar than around the pin 60 and between the pin and tension member socket. The provision of additional material in the bar toward the centre in the first rough drawing operation gives the requisite additional cross section of material 65 to enable the ribs 22 to be formed and yet

leave the body of the bar of the same thickness toward the centre as at the ends, as clearly shown in Figure 3.

Having thus described my invention, what I claim is;—

1. A process of making forged brake beam fulcrums, which comprises rough forging a straight bar to leave greater amounts of metal at the centre than at other points of the bar, and subsequently forming the 75 U-bend and tension member socket of the fulcrum from the increased amount of metal at the centre of the bar.

2. A process of making forged brake beam fulcrums, which comprises rough forging a 80 straight bar to provide greater amounts of metal at certain points therein, and subsequently forging the bar to form fulcrum pin bearings and stiffening ribs of said additional amounts of metal, meanwhile leaving the thickness of the bar body uniform 85 throughout its length between the centre portion and ends.

3. A process of making forged brake beam fulcrums, which comprises displacing metal 90 at the centre of a bar to form a U-bend located out of the plane of the bar, and dividing the bar into two aligned arms and subsequently bending the arms into parallelism.

4. A process of making forged brake beam fulcrums of U-shape, which comprises forging a bar intermediate its ends to form a U-bend located out of the plane of the bar, and simultaneously forming a brake 100 beam tension member socket in said bent portion forming the bar on either side of the bend to the desired shape, and finally bending the portions into parallelism.

5. A process of making forged brake beam 105 fulcrums, which comprises forging a brake beam tension member socket at the centre of the bar, forming the bar on each side of said socket to the desired shape, and finally bending the bar at points adjacent the socket to 110 form a U-shaped structure.

6. A process of making forged brake beam fulcrums which comprises offsetting the end portions of a bar in opposite directions, twisting the ends of said bar at the offsets, 115 and bending the bar to U-shape.

7. A process of making forged brake beam fulcrums, which comprises drawing out a bar to form portions of different width thereon, forging the drawn out bar to form arms 120 of uniform thickness and projections from said arms built up of the greater amounts of metal in the wider portions of the drawn bar, and bending the forged bar at points adjacent its centre.

8. A method of making forged brake beam fulcrums, which comprises increasing the stiffness of a bar at the centre and in portions on each side of the centre, leaving portions of less stiffness between the centre and 130

said stiffened portions in which the bar is bent to dispose the centre out of the plane of the rest of the bar, and forming said centre to receive a brake beam tension member and to fix the distance between the arms of the finished fulcrum and subsequently bending the bar at the unstiffened points adjacent the centre.

9. A process according to claim 8, characterized by twisting the bar adjacent its ex-

tremities before bending, and bring the edges of the bar beyond the twists into alignment without placing a greater fiber stress in one edge of the bar than in the other by oppositely offsetting end portions of the bar 15 prior to twisting.

In witness whereof, I have hereunto set my hand.

ERNEST R. VIBERG.